

May 12, 1936.

J. E. THORNTON

2,040,575

METHOD FOR THE PRODUCTION OF COLOR CINEMATOGRAPH FILMS

Filed March 31, 1934

3 Sheets-Sheet 1



Fig. 1.

INVENTOR

J. E. Thornton  
by J. O'uden O'Brien  
Attn.

May 12, 1936.

J. E. THORNTON

2,040,575

METHOD FOR THE PRODUCTION OF COLOR CINEMATOGRAPH FILMS

Filed March 31, 1934 3 Sheets-Sheet 2



J. E. Thornton  
by Jowden O'Brien  
attu.

May 12, 1936.

J. E. THORNTON

2,040,575

METHOD FOR THE PRODUCTION OF COLOR CINEMATOGRAPH FILMS

Filed March 31, 1934

3 Sheets-Sheet 3



Fig.10.



Fig.14



Fig.15.



Fig.13.



Fig.16.

INVENTOR

J. E. Thornton  
O. O'wen O'Brien  
Atty.

## UNITED STATES PATENT OFFICE

2,040,575

METHOD FOR THE PRODUCTION OF COLOR  
CINEMATOGRAPH FILMS

John Edward Thornton, Jersey, Channel Isles

Application March 31, 1934, Serial No. 718,440  
In Great Britain April 5, 1933

3 Claims. (Cl. 95—2)

This invention relates to cinematographic films with sound and picture records in parallel rows, and provides means whereby such records, first formed in black silver, can be changed or colored so that the picture records may be relief colloid images in one or more colors and the sound record be a relief colloid record in a different color, or black, the two records being formed simultaneously in separate rows, at the same operation or process, by applying to the black silver images of the two records a dry plaster of soluble colloid having stripes of differently colored colloid, or stripes of colored colloid and black colloid, followed by chemical action of a bleaching and hardening bath and other treatment.

Although the invention is designed more particularly for use in the production of multi-color pictures with sound on the same film, it can also be employed in the production of monochrome pictures.

The main feature of the invention consists in the means, method, and process for changing the images from black to color, and for producing differential coloring of the sound record and of the picture-records, both of which are formed parallel with each other upon the same film strip.

Throughout the following specification and claims the term "color" is used in its broadest sense as embracing any color including black.

The invention is applicable to films of the subtractive type, either in monochrome form, or in multi-color form of two, three, or four colors; and also to film-constructions in which the color-component images are all upon one face of a single-ply film, or upon two opposite outer faces of a single-ply film, or enclosed and protected between the supports of a two-ply cemented film.

According to the invention a cinematograph strip of positive images is produced by printing through a negative strip on to a positive strip of the ordinary type sensitized with gelatino-silver emulsion, then the film is developed fixed and washed, all in the usual manner, resulting in a strip having a series of positive images of metallic (or black) silver embedded in the gelatine and with the broad face of each image turned towards the outer face of the film and with the point or apex of each image turned towards the cellulose film support.

The image of the sound record is printed on the positive film alongside and in the margin of the picture records, and such image is developed and treated simultaneously with the picture records in the same manner, forming a sound

image of metallic silver also embedded in the gelatine. Although it is usual to have only one sound track, the invention can be applied to films having two or more sound records in different margins.

After development both kinds of records are in non-relief and non-colored, and are of metallic silver similar to an ordinary monochrome silver-print; and the method of their production up to this stage follows the standard practice usual for producing the ordinary black and white pictures.

One necessary condition of the invention (not required for ordinary films) is that the gelatine layer in which these metallic silver records are embedded must be sufficiently hardened to prevent its dissolving and washing away when the film is treated in warm water in the subsequent operation of relief development hereinafter described. In other respects the film and its sensitive emulsion are of standard type. This insoluble condition of the gelatine containing the silver image may be effected by suitable treatment during manufacture of the sensitive film, for example, by the addition of a small amount of chrome-alum to the emulsion before coating, or by treatment in a formaline bath after coating. Or instead, and in order to more definitely control the degree of insolubility, the film may be hardened after passing through all the developing, fixing and washing treatment, for example by passing the printed developed fixed film through a hardening bath of chrome-alum, formaline, or the like, and then washing and drying the film. Or alternatively, the hardening agent may instead be combined with the fixing bath, so that fixing and hardening are one operation only. Thorough washing is necessary to remove all soluble salts from the gelatine after any of these treatments. If however, the colored colloid is of the kind which only requires cold water for its solution, then the aforesaid hardened condition of the silver gelatine layer is not necessary.

Having produced a film with a sound record and a series of picture records in metallic silver, the next step is to color it.

According to the invention the first step of this coloring process is effected by adhering or cementing to the face of the developed film of metallic silver images (which are embedded in the layer of hardened gelatine) a multi-colored plaster in the form of a tape or ribbon, which comprises a layer of non-hardened soluble colored colloid, the said plaster being differently colored in stripes for the sound record and the picture

records. The second step consists in so treating the image of metallic silver by a bleaching-hardening bath, of the type hereinafter described, that a chemical re-action is set up which has 5 the effect of rendering insoluble such portions of the colored colloid of the plaster as are in contact with the silver image and of also permanently amalgamating them with or uniting them to the silver image layer, such insolubilization of 10 the colloid being in direct ratio to the amount of metallic silver contained in the image. The third step consists in dissolving and removing such parts of the colored colloid as still remain soluble and are not required for building a colored 15 image. The fourth step consists in entirely removing the silver salts from the film by dissolving them in a bath of sodium-hyposulphite or other solvent, followed by thorough washing to remove all salts. The result is that the unwanted 20 colored colloid and unwanted silver salts having been dissolved and removed, there is left behind only a colored colloid image in relief which is firmly adherent to the gelatine of the under layer, which latter has been rendered transparent 25 by the bleaching of the metallic silver.

Several variations in the aforesaid four steps can be made (hereinafter described under the heading of modifications), but retaining the governing 30 principles necessary to produce the finished article or cinematograph positive, which, when complete, comprises a strip of transparent cinematograph film support, an imageless silverless transparent colloid player attached to the support, and insoluble colored colloid relief images of a sound record and a series of insoluble colored colloid relief images of picture records, all being superimposed upon and permanently amalgamated with the face of the said insoluble colorless 40 layer.

One important feature of the invention consists in the means and method and process of so treating the image of the sound record that it shall differ from the images of the picture records. This is attained by forming the plaster in 45 two different colors of colloid, as parallel stripes, so that when laid upon and cemented to the printed developed film and subjected to the subsequent chemical treatment the plaster will apply 50 different colors to the picture records and the sound record. For example, the picture records may be colored, green, blue, red, yellow or the like, whilst the sound record is colored black, grey, or other desired color. Or, alternatively, the picture records may be colored 55 black, green, red, or other color, whilst the sound record is left uncolored or bleached and semi-transparent. The method of constructing the plaster to effect this differentiation is hereinafter 60 described.

#### *The colored plaster with different colored stripes*

The colored "plaster" itself is constructed in any of the following forms. The preferred one 65 is:—

*Form A.*—A strip of porous paper is coated upon one surface with a layer of suitable colloid mixed with suitable coloring matter in parallel stripes of different colors as hereinafter described. The 70 plaster-ribbon may be made as a wide web which is afterwards cut into narrow strips when dry; or the narrow ribbons themselves may be separately coated. Coating is effected by any suitable known apparatus; for example, wide webs are 75 preferably coated and dried by the apparatus

generally used for coating webs of paper or film with photographic emulsions, or with the apparatus used for sizing and enamelling paper webs. For ready-cut narrow paper ribbons suitable coating apparatus is that generally used for gumming and drying tapes; or a wet rubber belt running horizontally may be used to which the paper tape is squeegeed; or an adhesive belt may be used to which the paper tape is adhered by slight pressure; or the tape may be carried by a textile or perforated metal belt which passes over a long suction table, the paper being held to the belt by exhausting air from the suction table by a suction fan. In any of these methods the colored fluid colloid is deposited upon the paper web or 10 tape from a hopper, weir, slot or ductor roller having a scraping knife, all of which are known methods of coating. After the colloid layer has set the coated web or tape is then dried by passing through a drying chamber fed with filtered 20 and warmed air free from dust in the usual manner of coating processes.

For the colloid it is possible to use any one of several kinds, or mixtures of two or more, and among those which are more or less suitable may be mentioned gelatine, glue, fish-glue, albumen, casein, agar, gum arabic, and gum-tragacanth or dextrine. A good colloid is a mixture of glue and gelatine. Another is albumen and fish-glue. Another is gum arabic alone.

The preferred colloid is clear soft gelatine mixed with a small proportion of very clear glue. This is the colloid used in the description of the process hereinafter illustrated.

The coloring matter incorporated with the colloid must be extremely fine pigment, or a transparent pigment, or a dye-lake of a sufficiently transparent type, or a vat dye in colloidal dispersion, or an aqueous solution of a leuco compound or dyestuff, or any other coloring agent which is 40 sufficiently transparent and is also satisfactorily miscible with the particular form of colloid adopted. Two or more colors may be mixed to produce any intermediate shade, or any lower or duller tone desired.

The invention can be applied to films of various forms or types, as hereinafter described in detail under the heading of "different constructions" and for each of these a different arrangement of the color stripes of the plaster is necessary.

If the plaster is required for producing only one picture-color and sound it is made of single-width only. But if the plaster is required for applying two picture-colors and sound upon one 55 side of a double-width film it is made of double width, with the two colors coated side by side as parallel stripes. Or if the 2-color film is printed upon opposite sides, then two plasters of single-width are used, one being provided with sound 60 color. For 3-color work a triple-width plaster may be used having three colors applied in three parallel stripes, one being provided with sound color. Or alternatively a single-width and a double-width plaster may be used, one strip having sound color; or alternatively three single-width plasters may be used. For 4-color work a quadruple-width plaster may be used having four colors applied in four parallel strips; or alternatively, two double-width plasters; or alternatively four single-width plasters; in each of these 4-color arrangements a sound color is provided on one of the strips.

But whichever of these alternative arrangements is adopted, one of the plasters is provided

with a narrow stripe or edge differently treated from the rest of the coloring of the plaster and corresponding in location to the sound record in the margin of the film.

- 5 This different marginal stripe for the sound record is formed of colloid containing a different color, for example, black, grey or blue, which, when the entire plaster is laid over the film, covers only the sound track, whilst the other 10 coloring matter covers only the picture records. When a film covered by such plaster is treated by the chemical processes hereinafter more fully described, it eventually emerges with its picture records in color and its sound record in black, 15 grey, blue or whatever may be chosen.

In some films two or more sound records are required, and in such cases a corresponding number of differently-colored colloid sound stripes are formed on the plaster.

- 20 In another arrangement of the plaster a black color for sound can be got by coloring the sound record in one color such as red, and covering it with a green blank space on the opposite side of the film, the green and red forming black when 25 superimposed.

Although the film-strip is perforated in the usual manner for registration and traction purposes, the plaster tape need not necessarily be perforated, as it can be laid over the film by 30 machine with sufficient accuracy to ensure that the differently colored tracks shall lay correctly over their own portions of the images. If, however, greater accuracy is desired, the plaster tape may be perforated in both margins similarly to 35 the film itself. Or it may be perforated in only one margin, the one next to the sound track. These perforations in the plaster tape will have the effect of very accurately placing and superimposing the sound track of the plaster on to the 40 sound track of the film.

The alternative forms of plaster, and methods of their construction, are as follows:—

*Form B.*—For this a paper backing is used which has been waterproofed and is therefore 45 non-porous. It may be prepared by impregnating porous paper with hot wax or with an oleate of a fatty acid. Or it may be prepared with a coating of rubber solution. Or with a coating of shellac or other resin. The colored colloid is 50 coated upon this prepared paper in the manner previously described.

The plaster is adhered to the face of the printed film by slightly moistening and softening the surfaces of gelatine film and colored colloid, then 55 squeegeeing together between rolls, and afterwards the dry paper backing is pulled off or stripped, leaving the colored colloid firmly attached to the printed gelatine film.

The mode of manufacturing such a plaster is 60 similar to that used in the manufacture of the well-known stripping films which were formerly in common use but are now almost obsolete.

*Form C.*—In this form of plaster no paper backing is used, and it consists entirely of colored 65 colloid alone. This is manufactured in web or tape form by casting or flowing the liquid colored colloid on to a polished moving surface, whereon it is allowed to set and dry, and from which it is finally stripped and then slit or trimmed and 70 reeled for storage and use. The moving surface is preferably an endless belt of polished metal, or a continuous belt of polished celluloid, or a belt of paper or the like which has been coated with celluloid solution or with a resinous varnish to 75 give it the necessary glossy surface. A metal

drum or other polished surface may be used for short lengths only.

This colloid plaster is applied to the printed film and otherwise handled and treated in the same manner as the previously described forms 5 of plaster A and B.

#### *General procedure or routine of operations*

The method of producing colored films according to the invention requires the following 10 operations and sequence. They are described as applied to the production of a 2-color film having differently colored images upon opposite sides.

The film to be printed, which is sensitized upon both sides, is first perforated with suitable 15 perforations for registrations and traction purposes.

It is then printed in any known manner, but preferably from a double-width negative by optical projection in a printing machine as shown in the specification of my British Patent No. 20 373,312, which produces a pair of prints simultaneously, and in accurate registration one with the other, upon opposite sides of a film sensitized upon both sides with gelatino-silver emulsion. Other methods of printing the film may however 25 be employed.

The double-sided printed film is then developed, fixed, washed and dried in any known type of developing machinery.

The two plasters of different colors are then 30 cemented applied to opposite sides of the film in perfect optical contact therewith in the manner aforesaid and the film, together with its plasters, is passed into the bleaching bath.

The bleached film is next passed into the colloid-dissolving relief-developing apparatus, from which it emerges as a film having pairs of differently colored reliefs or color-component images upon opposite sides, thus producing a complete 2-color film, which is next fixed in a sodium-hyposulphite bath to dissolve the remaining silver-salts, after which the film is washed and dried.

*The machine and processes.*—The plaster may be adhered to the surface of the developed film in several ways. The preferred way, which is very simple in operation, is carried out in the machine illustrated in the accompanying drawings Fig. 1, where a film with two images upon opposite sides is shown in the process of being 50 colored by two plasters applied to opposite sides.

The film (which has been printed, developed, washed and dried, and which carries picture records and sound record formed of metallic silver) is carried on a supply roll F from which 55 it is drawn off by sprocket feed rolls f<sup>1</sup> which engage with its perforations, and in its movement is passed through a damping trough and rolls F<sup>2</sup> by which its gelatine surface is made sufficiently damp, soft and tacky.

It is then led between two multi-colored tape or ribbon plasters 2 and 3 which are in turn drawn off supply rolls L<sup>1</sup> and L<sup>2</sup>. The colored colloid of these plasters is dry, but very absorbent, and preferably comprises more or less glue which strongly adheres to the damp film surface and the two become physically united or amalgamated.

In a modification the gelatine of the film may be impregnated with a dilute solution of glue, 70 glycerine, and water to give it better adhesion as well as softer characteristics.

The three ribbons 1, 2 and 3 next pass between a set of pressure rolls A<sup>1</sup> and B<sup>1</sup> mounted on weighted frames A and B by which the two glue- 75

colloid faces of the plasters 2 and 3 are squeegeed into perfect optical contact with the faces of the gelatino-silver-images, and complete adhesion of the glue-colloid to the gelatine-silver image is effected. The number of rolls used may be more or less than shown according to speed of production desired.

One of the frames together with its rolls is mounted with a floating movement controlled by 10 the weighted arms.

The purpose of this is to ensure that the pressure upon the plasters will always be the same however much they may vary in thickness, and thus prevent variable squeegeeing and too much 15 or too little pressure. It also provides for using two or three bands yet always with the same pressure.

The triple ribbon then passes through a drying chamber K fed with warmed air at a temperature only high enough to dry out some of the moisture but not to melt the colloid.

The triple ribbon then passes into and through a bath M<sup>1</sup> containing the bleaching solution, which quickly penetrates the porous paper backings, passes through the colored colloid layers, and attacks the silver in the layers of hardened gelatine of the film, until the silver images are completely bleached and the colored colloid where in contact with such images is rendered 30 insoluble and becomes amalgamated with the hardened gelatine of the bleached silver image layer.

At this stage therefore the two kinds of image are amalgamated or interlocked by the chemical 35 reactions and insolubilization of the gelatine and colloid of each kind of image in proportion to the original quantity of metallic silver involved in the reaction.

The triple ribbon with its bleached images 40 then passes into a colloid-dissolving bath M<sup>2</sup>. In this bath the soluble parts of colored colloid not required to form parts of the colored images are dissolved and washed away, leaving behind on the film a series of colored colloid images which are in relief. As the ribbon emerges 45 from this bath the two paper supports are stripped away by rollers M<sup>2</sup> and M<sup>3</sup>.

The film (now a single ribbon) with its colored relief images, then passes into another bath M<sup>3</sup> 50 containing the fixing solution which dissolves and removes the remaining soluble salts of silver, leaving a layer of original insoluble gelatine free from any trace of the original silver images, upon which are superimposed and amalgamated clear 55 and transparent images of pure colored colloid in relief.

The film is then passed into a washing tank M<sup>4</sup> by which the fixing solution is washed out of the colored colloid images and out of the 60 transparent hardened gelatine layer beneath them. As a final precaution the washed film may be passed through a supplementary final washing tank M<sup>5</sup> though this is not absolutely necessary.

Or it may be treated in the bath and sprays N 65 with a hardening and flexing solution of alum and glycerine, or with a cellulose varnishing solution either by this final tank M<sup>5</sup> or by the spraying devices N or by both in combination.

The film then passes into and through a drying chamber P fed with warm filtered air, and when dry is reeled at P<sup>1</sup>.

The foregoing description of coloring by two plasters applies when the film is required with 75 colored images upon opposite sides.

Several other variations are possible in the method of applying the multi-color plaster and bleaching solution to the printed images of metallic silver, and are hereinafter described in detail under the heading of "modified details and routine".

If the film requires coloring only upon one side, one plaster only is used, the rest of the procedure being the same.

*Bleaching and hardening bath.*—The type of 10 bleaching and hardening is that commonly known as ozobrome, carbro, or any other similar type. Many modifications in the ingredients and proportions of such baths have been published, and the invention is not limited to the use of 15 any particular one. They usually comprise a mixed solution of a soluble bichromate and a ferricyanide or a copper salt; and sometimes in addition to these substances soluble bromides are 20 present in the solution. The effect of such a bath 25 is that the metallic silver of the image is transformed into a silver salt, and the gelatine, where in contact with the metallic silver, is tanned, hardened or insolubilized to an extent in exact proportion to the quantity of metallic silver forming 30 the image. Therefore, according to this process the amount of silver in the film-image definitely controls and regulates the quantity of colored colloid that will be rendered insoluble and will attach itself to the silver image, and therefore the silver also controls the quantity of such 35 colored colloid that will be left soluble to be dissolved and removed by the dissolving bath. In this way, by careful control of the amount of metallic silver in the primary image in the lower 40 layer of insolubilized gelatine, by suitable adjustments of the length of exposure, time of development, and strength and composition of the developer, it becomes possible to control exactly the amount or depth of color of the secondary 45 image of insoluble colored colloid image in the upper layer. After removal of all the silver, the whole of the gelatine of the lower layer, including the parts where there had been a silver image, 50 becomes transparent, and after removal of the unwanted surplus colored colloid of the upper layer by its solvent bath there is left a relief image of transparent colored colloid only which is superimposed upon and united to an imageless layer of non-colored transparent insoluble or hardened gelatine.

#### *Modifications in details and routine of operations*

There are quite a number of possible modifications in practice of the operations that will 55 produce similar finished results, for example:—

*The colloid and its solvents.*—In the foregoing description it is assumed that a colloid is used which requires heat for its solution before coating and is set by cooling and is dried by warm 60 air after coating. Such a colloid is gelatine, or glue and gelatine. For developing such colloid into relief warm water is therefore used.

But alternatively, a colloid may be used which is soluble in cold, and is solidified and dried by 65 the application of warm air after coating. Such a colloid is gum-arabic, fish-glue, and others of those hereinbefore mentioned. For developing such colloid into relief cold water or other cold solvent is therefore used.

*Silver solvents.*—The ordinary bath of sodium-hypo-sulphite may be used for dissolving the remaining silver salts. Or any other suitable substitute that will easier attack the silver imprinted 70 in the hardened gelatine, such as the well- 75

known "ferricyanide and hypo" bath, or the like. Other modifications of treatment are as follows:—

(1) Hardening of the colloid layer carrying the silver image may be affected during manufacture of the sensitive material. Or it may be effected after manufacture but before printing, by passing the sensitive strip through a bath of chrome alum or formaline, then 10 drying. Or where it is desired to bleach after fixing the hardener, such as potash alum may be added to the fixing bath. In any case it is absolutely essential the gelatine of the silver image colloid layer should be rendered sufficiently 15 hard to prevent its solution in the warm water bath, and instead leave it permanently anchored to the cellulose support of the film.

(2) The printed gelatino-silver layer (if too hard owing to its having been dried after development) may be slightly softened to ensure better adhesion, by passing it through a weak alkaline bath, for example, one containing ammonia or sodium. The colored colloid of the plaster may or may not be treated in the same way, according 25 to requirements. The addition of a little glycerine is useful. The addition of glue hereinbefore referred to may also be made to this softening bath if desired.

(3) The bleaching bath, which serves the double purpose of bleaching the metallic silver and of rendering insoluble such portions of the colored colloid as are in contact with such silver, may be applied at either one of different stages.

The preferred method is to adhere the dry 30 plaster to the printed gelatine surface of the film which has first been slightly softened by an alkaline bath, and then apply the bleacher by passing the complete film with its adherent plaster through the bleaching bath, for a sufficient 40 time to allow the solution to penetrate firstly the porous paper support and secondly the colored layer and the silver-image layer, and to thus effect a complete bleaching of the silver therein and effect complete insolubilization of the 45 colored colloid in contact with such silver.

(4) Bleaching and hardening of the image may be effected by one combined bath at one operation.

(5) Bleaching and hardening of the image may be effected by two separate baths applied in succession at two separate operations, thus allowing more variations of control of the hardening operation according to the kind of gelatine used.

(6) Bleaching of the image may be effected by incorporating the ingredients of the bleaching bath with the colored colloid before it is coated on to the paper support of the plaster, or by soaking the colored plaster in a bath of bleaching solution and then drying the plaster. When 60 bleaching it is then only necessary to bring one dry strip into pressure-contact with the damp strip to produce a liquid bleacher in situ.

(7) Bleaching can be effected by soaking the printed film until its gelatine is saturated, in a 65 bath of chromic acid, then applying the dry plaster to the film after the surplus solution has been removed from the surface.

(8) Bleaching may take place last of all, after fixing.

(9) Softening can also be effected by incorporating an alkali with the colored colloid of the plaster to become active only when damped.

(10) Good optical contact between the two gelatine surfaces (film and plaster) may be obtained if they are squeezed and adhered whilst

both surfaces are under water passing between immersed rolls so placed and constructed that any enclosed air is driven off at the edges. To effect this the position of the two supply spools of plaster needs changing to the position near the 5 spool F.

(11) Other porous materials than paper might be used as the support for the colored colloid in construction of the plaster, provided they are sufficiently porous to allow penetration of liquids 10 through the plaster to the silver. One such material would be a strip of cellulose xanthate, better known as cellophane or viscose, upon the face of which the colored colloid would be coated; or the strip squeegeed into contact with the wet colored 15 colloid whilst on its preparatory support and dried thereon.

(12) In another modification the backing of the plaster may be entirely dispensed with, the colored gelatine or other colloid being itself cast 20 in the form of a tape, or cut as a ribbon from a wide web of such material, as herein-described.

(13) The print may be fixed, washed, and dried, after leaving the developing bath. Then stored for coloring at any subsequent period desired. This is the preferred method and in the drawings showing the coloring processes and machinery therefor it is assumed that the already printed developed dried film is stored upon the supply spool F. 30

(14) The several processes may be combined in one set of machines as one continuous process. In such case after development the plaster is applied, bleaching follows, then fixing, washing and drying. Therefore the wet film passes 35 straight from the developing machine (without intermediate treatment or drying) and enters the coloring machine at the point where it makes contact with and between the two dry surfaces of the two plasters. In such case the damping F<sup>2</sup> 40 and preliminary drying K are cut out.

(15) Or the processes may be divided into two groups, carried out by two sets of machines, development, washing and drying being one process; and plastering, bleaching, fixing, washing 45 and drying a separate process. The advantage of this latter division is that it enables the coloring and finishing processes to be carried on entirely in a daylight room instead of an extension of the developing room. This is the preferred 50 method illustrated by the drawings.

(16) Where the stages of treatment are varied, as in modifications 3 to 8, the tanks and sections of the machine illustrated in the drawings are transposed or otherwise modified to suit such 55 variation of the preferred practice illustrated.

(17) Other modifications may be made in the arrangement of the machine. For example, very soft and adhesive layers may be sufficiently well adhered with only one or two pairs of pressure 60 rolls. But where the film surface is hard a number of pairs of rolls are required to ensure perfect adhesion. The rolls may be arranged horizontally, instead of vertically as shown in the drawings. The plaster tape supply spools L<sup>1</sup> L<sup>2</sup> may be placed between the damping apparatus F<sup>2</sup> and the pressure rolls if arranged horizontally immediately after the damping apparatus. The drying chamber K may be placed after the pressure rolls and before the bleaching tank M<sup>1</sup>, 70 between the two.

#### *Different constructions of films*

Another feature of the invention is the adaptability of the process to the production of cine-

matograph positives of different types or constructions, as illustrated by the following examples:—

- (A) A monochrome film having positives of one color only on one face of the film, for example black or sepia or blue, thus dispensing with all troublesome toning processes; and provided with a sound record in black, or color, formed alongside the colored picture records.
- 10 (B) A two-tone monochrome film, having positives in a deep shade of one color, for example sepia, on one side of the film; and on the other side partial positives in a lighter shade of the same color; and a sound record in black or color alongside.
- 15 (C) A two-color film having on one side complete positives in black, and on the other side partial positives in blue or red. By this means pictures with moonlight or night effect can be produced by blue and black, and pictures with sunset effects can be produced with red and black and with sound record in black or color alongside. Thus troublesome toning operations to obtain double-tones are abolished.
- 20 (D) "Plaster-relief" effects can be produced by "printing through" a film which is sensitized on both sides, the image depths being so regulated that the light background is printed upon one side only of the film, and the darker objects, such as furniture, figures of actors, trees, buildings, or the like are printed through on to both sides and thus receive a double quantity of color. Or the light parts may be printed upon one side and the dark parts upon the other side and each provided with different shades or intensities of coloring, and a sound record in black or color alongside.
- 25 (E) A multi-color film of 2-color type such as orange-red and blue-green can be formed with the two colors upon opposite sides of the film, each printed from different color-separation negatives which form pair-parts of the same picture, and a sound record in black or color alongside.
- 30 (F) A multi-color film of 2-color type (as in E) can be formed by printing the two pair-parts side by side upon a double-width film which, after coloring, is slit longitudinally and the parts superimposed and cemented together, and a sound record in black or color alongside one of the colors.
- 35 (G) A multi-color film of 3-color type can be produced by making two images, for example red and blue, in the manner already described, and then adding a third color such as yellow by re-sensitizing and re-printing over one of the other colors, by any of the various well-known methods. Or the third color may be formed first and another color over it. Or the third color can be added by photo-mechanical printing methods or by stencil methods, or in any other known way, and a sound record in black or color alongside one of the colors.
- 40 (H) A multi-color film of 4-color type can be more readily constructed according to this invention than by any of the methods previously known and described in some of my own published 4-color processes such as British specification No. 224,569 and its several divisions and associated specifications. The simplest way of forming such a 4-color film by use of the present invention is by printing two component images (of a set of four) side by side upon one face of a sensitive film in one emulsion, and the other two images of the set side by side upon the opposite face of the film in another emulsion. The four images are printed and developed simultaneously by known methods

to form groups of four silver images, and are afterwards colored by adhering to one face a plaster comprising two parallel stripes of differently colored colloid, and to the other face another plaster comprising two other parallel stripes of differently colored colloid. By this means all four images are simultaneously colored at one operation as the film is passed through the various baths. A sound record in black or color is formed alongside one of the colors. After printing and 10 coloring the double-width film is slit into two single-widths, which are then superimposed and cemented together with sound images inside as in my British specifications Nos. 232,302 or 246,282. This 4-color film is produced substantially as described in my British specification No. 224,573, upon double-width film-material of the type described in my British specification No. 233,985, but its coloring is effected by the improved method described in the present invention 20 instead of by the methods described in the specification aforesaid, and a sound record black or color is added alongside.

This invention is also applicable for coloring a multi-color film of the type described in my British specifications Nos. 285,227 and 285,228 in which the film is made of insoluble gelatine without any cellulose support. The construction methods are the same, but with the coloring effected according to this invention instead of by the methods therein described; and the film-material of that film (which consists of gelatine plus a gelatino-silver emulsion and no cellulose support) is itself non-colored before printing, and is only colored (after the silver images have been 35 formed) by the process according to the present invention. A sound record in black or color alongside is also added.

In all these examples the sound record is differently treated or colored from the picture records, by suitable construction of the multi-color plaster as hereinbefore described.

Figs. 2 to 16 of the accompanying drawings will enable the invention, and its differences from previously known processes, to be readily understood. In these drawings:—

Fig. 2 is a transverse section through a sensitized film before exposure, 1 being the transparent celluloid support, 2 the adhesive substratum, and 3, the sensitized silver emulsion layer of insoluble gelatine;

Fig. 3 is a similar section after exposure and development showing images of metallic silver in the gelatine layer 3, the images 3<sup>a</sup> being the sound record of metallic silver and 3<sup>b</sup> the picture records of metallic silver.

Fig. 4 is similar section showing the colored plaster 4 with its paper backing 5 adhered to the face of the insoluble gelatine layer 3 with the developed images 3<sup>a</sup> and 3<sup>b</sup> of metallic silver embedded therein.

Fig. 5 is a similar section of the finished positive showing the transparent color picture records 3<sup>c</sup> in relief and black sound record 3<sup>d</sup> in relief after the unwanted silver and the unwanted colored colloid of the layer 3 have been dissolved and removed.

Fig. 6 is a perspective view showing the colored plaster 4 with white paper support 5 being applied to the metallic silver images embedded in the hardened gelatine layer 3 after the film has passed through the developing bath and before passing to the bleaching bath, the plaster 4 having a wide orange red stripe 4<sup>a</sup> for coloring the picture rec-

ords and a narrow black stripe  $4^b$  for the sound record.

Fig. 7 is a perspective view showing the paper backing 5 of the plaster 4 being stripped from the film after the latter has passed through the bleaching bath, the colour having been left on the film, and before the surplus unwanted colored colloid has been dissolved and removed.

Fig. 8 shows the final finished film in which the unwanted colored colloid has been dissolved and removed, leaving black colored colloid on the sound image  $3^a$  and orange-red colored colloid on the picture images  $3^b$ . The metallic silver has also been dissolved and removed, leaving images of transparent insoluble colloid in place of the black-silver, with the colored colloid images superimposed upon and firmly amalgamated with the insoluble colloid parts of the lower layer of insoluble transparent gelatine. These colored colloid images are in relief, and stand above the lower layer of gelatine, to which they are permanently united or amalgamated as shown in Fig. 5.

Figs. 9 and  $9^a$  show how a 2-color film is made with orange-red picture component images upon one face and blue-green picture-component images upon the opposite face, and black sound record not shown alongside either the red or green picture records. Fig. 9 being a longitudinal section of the film with developed metallic silver images  $3^a$  on each side and colored plasters 4 adhered thereto and Fig.  $9^a$  being the finished 2-color film with orange-red and blue-green relief images upon each opposite sides forming complete 2-color picture records the black sound record being formed parallel therewith in the margin of the film. The finished film comprises a transparent central support 1 of celluloid, two layers 2 of adhesive substratum 2, two layers 3 of insoluble transparent imageless silverless gelatine, an insoluble colloid relief and picture  $3^a$  on one face and an insoluble colloid relief green pictures  $3^b$  on the other face.

Figs. 10, 11, 12 and 13 illustrate the steps in forming the 2-color film Fig. 13; this is produced from the double-width printed film Fig. 10 which shows the developed black metallic silver images; the paper backed colored plaster Fig. 11 adhered to the silver images; Fig. 12 shows the film with its colored colloid relief images, and Fig. 13 the finished film with the two parts slit and then cemented together face to face; (or they may be cemented back to back, or face to back).

Fig. 14 shows a multi-color plaster 4 for a 2-color and sound film having three colored stripes;  $4^a$ , being for the black sound record and  $4^b$ ,  $4^c$  for the two color-picture records respectively.

Fig. 15 shows a multi-color plaster 4 for a 3-color and sound film having four colored stripes;  $4^a$  (black)  $4^b$  (magenta)  $4^c$  (yellow) and  $4^d$  (blue) for the black sound record and the three colored picture records respectively.

Fig. 16 shows a pair of multi-color plasters for producing a four-color and sound film built up of two double width films; the first plaster has 3 colored stripes  $4^a$  (black) for the black sound record,  $4^b$  (red) and  $4^c$  (yellow) and the second plaster two colored stripes  $4^d$  (blue) and  $4^e$  (green). They may be printed as one strip or be slit into two strips. In assembling the red stripe goes over the green stripe and the yellow over the blue.

Instead of the tape or plaster being of the same width as the film a narrow tape or plaster may be employed provided with a layer of colored

colloid the width of the picture records only, so that when applied to the face of the printed film the picture records are colored but the sound record is not colored since the plaster leaves it entirely exposed. The sound record is thus differentially treated from the picture records and may be finished either as black silver or as colorless bleached silver.

In producing such film an ordinary positive film sensitized with gelatino-silver-emulsion is exposed or printed under a negative having color records and under a negative having a sound record, which latter is printed parallel to the former. Both may be printed simultaneously.

It is next developed to produce images of both kinds of record in metallic silver. It is then washed, after which the plaster tape or ribbon is applied to the silver picture images whilst the film is still wet.

Or if preferred the developed film may be fixed, washed and dried, after which the plaster tape or ribbon is then applied to the film by first wetting either the film or the plaster.

The plastered film is next treated in a bleach-hardening bath of well-known type by the chemical action of which the silver is bleached and the colored colloid is rendered insoluble wherever in contact with silver and in exact proportion to the amount of silver present in the image.

The bleached image is then treated in a solvent by which the surplus colored colloid not used to form the image is dissolved and removed. It is also treated in a solvent by which the silver salts are dissolved and removed, leaving behind a film which comprises a transparent support, a transparent imageless layer of insoluble gelatine attached to the support, and a relief image of colored colloid superimposed upon and standing above the transparent gelatine layer, representing one of the color parts of the picture-record.

If it is desired to form the sound record in black metallic silver it is coated with a narrow stripe of protective varnish after development fixing washing and drying, in order that the black silver may be protected from the bleaching bath in the subsequent operation and therefore remain black permanently. Or such protective layer may be a strip of adhesive waterproof tape (such as rubber covered plaster). Either the protective varnish or protective tape may be applied to the film before development or after development and drying.

But if it is desired to form the sound record with a colorless image, such protective layer is omitted and the sound record is bleached at the same time as the picture record and the silver is dissolved and removed in the fixing bath as aforesaid.

After all operations aforesaid have been completed the film is washed and dried.

What I claim as my invention and desire to protect by Letters Patent is:—

1. An improved process for producing a combined color picture and sound record cinematograph film having the picture records formed in relief in colloid of one color and the sound record in relief in colloid of another color, the two records in relief colloid being formed simultaneously from a film in which both records have first been formed by exposure and development as primary images of metallic silver embedded in a layer of hardened gelatine, the said process comprising the following steps in combination:—(a) applying in optical contact on to the aforesaid silver images a tape carrying parallel stripes of differ-

ently colored colloid mounted on a porous paper support applied to the film simultaneously, the stripe covering the picture areas being of one color and the stripe covering the sound record being of a different color; (b) passing the film and the colloid tape adhered thereto into a bleaching and hardening bath by the reaction of which the silver images are bleached and the colloid stripes are rendered insoluble whenever in contact with the silver of the images and in direct ratio to the quantity of silver in the images; (c) dissolving and removing all unwanted colloid and removing the porous paper support that has not become insolublized and amalgamated with the underlying silver image, thus producing relief images of insoluble colloid; (d) dissolving and removing by a fixing bath the unwanted silver salts thus producing a clear transparent imageless layer of gelatine upon which the aforesaid colloid relief images are superimposed; and finally washing and drying the film; thus producing a positive cinematograph film strip having a layer of imageless transparent gelatine firmly attached to its transparent cellulose support, and another layer comprising sound and picture records of colloid reliefs in parallel formation superimposed upon and firmly attached to the aforesaid imageless layer of hardened gelatine, the picture records being in colored colloid reliefs and the sound record being in a differently colored colloid relief, these colloid relief images being the only images left on the film.

2. An improved process for producing a combined color picture and sound record cinematograph film having the picture records formed in relief in colloid of two colors and the sound record in relief in colloid of a third color, the two records in relief colloid being formed simultaneously from a film in which both records have first been formed by exposure and development as primary images of metallic silver embedded in a layer of hardened gelatine, the said process comprising the following steps in combination:—  
(a) applying in optical contact on to the aforesaid silver images a tape carrying three parallel stripes of differently colored colloid mounted on a porous paper support applied to the film simultaneously, the stripes covering the picture areas being of two different colors and the stripe covering the sound record being of a third color; (b) passing the film and the colloid tape adhered thereto into a bleaching and hardening bath by the reaction of which the silver images are bleached and the colloid stripes are rendered insoluble wherever in contact with the silver of the images and in direct ratio to the quantity of silver in the images; (c) dissolving and removing all unwanted colloid that has not become insolublized and amalgamated with the underlying silver image, thus producing relief images of insoluble colloid and removing the porous paper support; (d) dissolving and removing by a fixing bath the unwanted silver salts thus producing a clear transparent imageless layer of gelatine upon which the aforesaid colloid relief images are superimposed; and finally washing and drying the film; thus producing a positive cinematograph film strip having a layer of imageless transparent gelatine firmly attached to its transparent cellulose support, and another layer comprising sound and picture records of colloid reliefs in parallel formation superimposed upon and firmly attached to the aforesaid imageless layer of hardened gelatine, the picture records being in colored colloid reliefs and the sound record being in a differently colored colloid relief, these colloid relief images being the only images left on the film.

upon which the aforesaid colloid relief images are superimposed; and finally washing and drying the film; thus producing a positive cinematograph film strip having a layer of imageless transparent gelatine firmly attached to its transparent cellulose support, and another layer comprising sound and picture records of colloid reliefs in parallel formation superimposed upon and firmly attached to the aforesaid imageless layer of hardened gelatine, the picture records being in colored colloid reliefs and the sound record being in a differently colored colloid relief, these colloid relief images being the only images left on the film.

3. An improved process for producing a combined color picture and sound record cinematograph film having the picture records formed in relief in colloid of a plurality of colors and the sound record in relief in colloid of a different color from any of the colors forming the picture records, the two records in relief colloid being formed simultaneously from a film in which both records have first been formed by exposure and development as primary images of metallic silver embedded in a layer of hardened gelatine, the said process comprising the following steps in combination:—  
(a) applying in optical contact on to the aforesaid silver images a tape carrying a plurality of parallel stripes of differently colored colloid, mounted on a porous paper support applied to the film simultaneously, the stripes covering the picture areas being of a plurality of different colors and the stripe covering the sound record being of a different color from any of the colors of the stripes covering the picture areas; (b) passing the film and the colloid tape adhered thereto into a bleaching and hardening bath by the action of which the silver images are bleached and the colloid stripes are rendered insoluble whenever in contact with the silver of the images and in direct ratio to the quantity of silver in the images; (c) dissolving and removing all unwanted colloid that has not become insolublized and amalgamated with the underlying silver image, thus producing relief images of insoluble colloid and removing the porous paper support; (d) dissolving and removing by a fixing bath the unwanted silver salts thus producing a clear transparent imageless layer of gelatine upon which the aforesaid colloid relief images are superimposed; and finally washing and drying the film; thus producing a positive cinematograph film strip having a layer of imageless transparent gelatine firmly attached to its transparent cellulose support, and another layer comprising sound and picture records of colloid reliefs in parallel formation superimposed upon and firmly attached to the aforesaid imageless layer of hardened gelatine, the picture records being in colored colloid reliefs and the sound record being in a differently colored colloid relief, these colloid relief images being the only images left on the film.

JOHN EDWARD THORNTON. 65